# EUROPEAN PATENT SPECIFICATION

(11) **EP 0 420 868 B1**
(45) Date of publication and mention of the grant of the patent: **15.09.1993**
(21) Application number: 89906387.9
(22) Date of filing: 17.05.1989
(51) Int. Cl.: C10M 133/38, C10M 133/40, C10L 1/22

(54) **METHOD OF FOR REDUCING WEAR ON SURFACES SUBJECTED TO FRICTIONAL FORCES**
VERFAHREN ZUR REDUZIERUNG DES VERSCHLEISSES AUF OBERFLÄCHEN, DIE REIBUNGSKRAEFTEN AUSGESETZT SIND
PROCEDE DE REDUCTION D'USURE SUR DES SURFACES SOUMISES A DES FORCES DE FROTTEMENT

(30) Priority: 18.05.1988 GB 8811696
(43) Date of publication of application: 10.04.1991
(73) Proprietor: BRITISH TECHNOLOGY GROUP LIMITED, London SE1 6BU (GB)
(72) Inventor: FODOR, Josef, H-1016 Budapest (HU); SCHOFIELD, Jack, Merseyside L49 6NP (GB)
(74) Representative: W.P. Thompson & Co.
(86) International application number: GB8900530
(87) International publication number: WO8911518

## Description

The present invention relates to a method of reducing wear on surfaces subjected to frictional forces, particularly between moving surfaces.

The primary purpose of lubrication is separation of moving surfaces to minimise friction and wear. Several distinct regimes are commonly recognised in the field of lubrication. Thus in fluid film lubrication the load is supported entirely by pressures within the separating fluid film. This film pressure is frequently generated by relative motion of the surfaces involved, which pumps the lubricant into a converging, wedge- shaped zone. The hydro dynamic behaviour of such bearings is completely dependent on the viscous behaviour of the lubricant. Both the load-supporting oil film pressure and the power loss are functions of lubricant viscosity in combination with the geometry and shear rate imposed by the bearing operating conditions.

As the severity of operating conditions increases, a point is eventually reached where the load can no longer be carried completely by oil-film support. High spots, or asperities of the mating surfaces must then shear with the lubricant in load support and the lubrication regime shifts from full-film to mixed-film and then to complete boundary high load, low speed, low viscosity lubricant, misalignment, high surface roughness or an inadequate supply of lubricant. With boundary lubrication, chemical additives in the lubricating composition and chemical metallurgical, and mechanical factors involving the two rubbing surfaces will determine the extent of wear and the degree of friction.

Under boundary conditions of lubrication, metal contact through the oil film results in junctions of asperities and subsequent metal tearing on a microscopic scale. As loads increase these contacts become more frequent and result in more plastic deformation, higher temperatures and welding with seizure eventually occurring on a gross and devastating scale. Hypoid gears, since they impose severe sliding conditions in combination with high contact stress are particularly susceptible to this type of damage. The organic lubricant film normally present becomes ineffective under the intense heat which leads to very high surface temperatures.

To combat welding under such extreme conditions, extreme pressure lubricants were developed. Such lubricants contain additives which react at the high contact temperatures to form high-melting inorganic lubricant films on the metal surfaces which prevent massive welding and breakdown. Generally, these additives consist of sulphur, chlorine, phosphorus and lead compounds which act either by providing layers of low shear strength to minimise metal tearing or by serving as fluxing agents to contaminate the metal surface and prevent welding. Since all extreme-pressure additives are affected by chemical action, i.e. the formation of covalent bonds, their use is generally avoided to eliminate possible corrosion difficulties.

Dry sliding, which involves solid-to-solid contact, not infrequently exists, even when adequate fluid film lubrication is provided. Dry sliding can occur for example, in starting up of a machine, with misalignment or inadequate clearance during run-in, during reversal of direction, and during any delays or interruptions in supply of the lubricating fluid. Where conventional oils and greases cannot be used because of extreme temperatures, high vacuum, radiation, or contamination, thin coatings of dry lubricants have been applied to reduce the higher friction and more extensive wear which otherwise obtain on rubbing the structural materials against each other.

Thus the goal of lubrication is elimination of this wear and minimising of friction which would otherwise be encountered in dry sliding. Whilst this can be accomplished by complete separation of the rubbing surfaces as by a full film of fluid lubricant, generally such complete separation is not possible under all working conditions and as a result, surface chemical effects have been brought into play in boundary lubrication to reduce friction and wear which does occur in boundary lubrication. Thus anti-wear agents have been added to liquid lubricants which produce a surface film on the sliding parts by either a chemical or physical adsorption mechanism, the film reducing friction and wear under boundary lubrication conditions.

A wide variety of compounds have been used for improving lubrication under boundary film conditions. Thus compounds containing oxygen such as fatty acids, esters and ketones, compounds containing sulphur or combinations of oxygen and sulphur, organic chlorine compounds such as chlorinated waxes, organic sulphur compounds such as sulphurised fats and sulphurised olefines compounds containing both chlorine and sulphur, organic phosphorous compounds such as tricresyl phosphate, thiophosphates and phosphites and also organic lead compounds have been used.

When the conditions in boundary lubrication are mild, polar additives having a polar group at one end of the molecule and a solubilising group at the other - usually a long chain hydrocarbon to effect solubilisation in the lubricating oil, have been used to provide an adherent adsorped film over metallic surfaces. A class of heterocyclic compounds useful as additives which provide friction modification and improved fuel economy are disclosed in WO 87/0596 and have the general formula: wherein Z is S, NR, PR or PRA, wherein A is 0 or S and R is H, alkyl, alkenyl, hydrocarbyl acyl, hydrocarbyl phenolate or -(CH₂)ₘQ, where m is 1 to about 12, and Q is O-alkyl or N-alkyl, X is independently H, COOH, NH₂ CONH₂, NHNH₂, OR, COR, NHR, OH, SH, or CN wherein R is the same as defined above; p is 0 to 2; e is 0 to 2 wherein e+p is 2 to about 4; T is NH₂, NHR wherein R is the same as defined above, SH, OH or their tautomers, hydrocarbyl acyl or hydrocarbyl phenolate; and Y is CN, C0₂ H or CH₂ NH₂ wherein A is the same as defined above. Such adsorped films of additive have hitherto only been successful under relatively mild boundary lubrication conditions, primarily because the thickness of such films is very low and usually of the order of one nanometer. Under more severe conditions of boundary lubrication, substances like tricresyl phosphate or zinc dialkyl dithiophosphates have been found necessary and in extreme rubbing conditions where severe metal-to-metal contact would otherwise be encountered, active sulphur, chlorine and lead compounds have been found essential. Such additives however react chemically to form low shear strength surface layers such as lead sulphide ion chloride or ion sulphide. This surface layer then prevents destructive welding, excessive metal transfer and severe surface breakdown. Such chemical reactivity with the surfaces of the sliding parts however is not in general desirable and is only undertaken when no other alternative is available.

As indicated, the polar type of compound which forms an adherent adsorped film over the moving surfaces is much to be preferred, but the thicknesses of such films which have been possible by the use of hitherto known additives in lubricating compositions have produced insufficient thicknesses of adsorped film to function under any conditions other than mild conditions.

US 3779920 discloses certain nitrogen-oxygen containing compounds in lubricating oil compositions comprising mineral oil of lubricating viscosity and at least one alkali metal and/or alkaline earth metal carbonate overbased sulphonate and/or phenate. These nitrogen-oxygen containing compounds are added to mop up the alkaline compound to prevent wear. In particular it discloses the use of 0.5% by weight hydroxyquinoline in one such composition.

SU 939527 discloses the use of 0.05 to 0.19% hydroxyquinoline in a composition also comprising a soapy plastics lubricant and copper. It is said that the alloying of the copper with the 8-hydroxyquinoline aids lubrication.

US 2030033 discloses the use of less than 1% dihydroxyquinoline as an inhibiter of gum formation in petroleum products.

US 3939084 discloses compositions for use as corrosion inhibitors. It is preferred that the compounds disclosed are used in amounts from 0.05 to 0.5% by weight. The most similar compounds to those of the invention include 4-6 dihydroxy pyrimidine each of which were used in amounts of 0.1 % by weight.

EP 69507 is concerned with additives which confer antioxidant and/or metal deactivating and/or electrical insulating properties. The heteroaromatic nitrogen containing compound most similar to those of the invention is 6-aminopurine which is used in an amount of 0.054% by weight.

It is an object of the present invention to provide a lubricating regime whereby adherent adsorbed films of polar material are provided up to 1,000 times thicker than have hitherto been possible.

The present invention concerns a radical advance in lubrication by providing a regime in which multimolecular layers are adsorbed onto the surfaces to be protected thus enabling comparatively thick protective films to be built up on sufaces subject to frictional wear. It has now been found that certain molecules have the property of forming such multimolecular layers when contacted with the surface as by incorporation in a carrier which is continuously or intermittently brought into contact with at least a portion of the surface to be protected. The molecules which have been found to have this property are essentially single or condensed unsaturated ring systems which comprise at least one six-membered unsaturated heterocyclic ring comprising at least one heterocyclic moiety which acts as a hydrogen acceptor, the molecule also comprising at least one hydrogen donor moiety. The molecules may comprise other five or six-membered unsaturated rings which together with the said six-membered unsaturated heterocyclic ring form a condensed ring system.

The multimolecular layers of the lubricating regime of the present invention are built up by initial adsorption of a layer of molecules onto the surface to be protected followed by adsorption of further molecules onto the initial layers to form a second layer and yet further adsorption to form more layers until films up to about 1 micrometer thick are formed. Without wishing to be bound by theory it is believed that presence of both hydrogen donor and hydrogen acceptor moieties in the heteropolar molecules enables this adsorption to take place.

Whilst unsubstituted heteropolar molecules are preferred substituents may be present on the heteropolar molecules provided they do not singly or collectively prevent interaction of the hydrogen donor and acceptor moieties as by steric hindrance. Thus, for example, hydrocarbon substituents such as alkyl groups should preferably not contain more than four carbon atoms, preferably not more than two carbon atoms. When the substituent is ortho to either the heteroatom or the hydroxyl group the steric hindrance effect is likely to be greater than when said substituent is in the meta or para position to either the heteroatom or a hydroxyl group. Alkene and alkyne substituents, carboxyl containing and amine containing substituents will all effect the activity of the heteropolar molecules and should be avoided.

In one embodiment of the invention therefore a method of reducing wear on a surface which is subject to frictional forces which comprises forming and maintaining on said surface a protective layer characterised in that said protective layer is a multi-molecular layer of a heteropolar compound comprising at least one unsaturated heterocyclic six-membered ring in which at least one wholly unsubstituted heteroatom moiety acts as a hydrogen acceptor and in which said compound also comprises at least one hydrogen donor moiety, and in which said heteropolar compound has no substituent which by itself or together with another substituent or substituents creates such steric hindrance and/or renders the molecule so basic or acidic or so alters the steric geometry of the molecule as to prevent interaction of the hydrogen donor and acceptor moieties of one molecule of the heteropolar compound with the hydrogen donor and acceptor moieties of another molecule of said heteropolar compound nor any substituent which by itself or together with another substituent or substituents has the effect of solubilizing said heteropolar compound in a selected carrier to the extent that migration of the heteropolar compound to the interfaces of the carrier with the carrier environment is prevented and in which the protective layer is formed on the surface to be protected by contacting at least a portion of the said suface with a composition comprising a carrier and dissolved and/or dispersed therein an effective amount of said heteropolar compound.

Formation of the multimolecular layer of heteropolar molecules may be effected by incorporating the heteropolar compound in a carrier which is brought into contact with the surface to be lubricated. It has been found that the heteropolar molecules migrate through the carrier onto the surface to be lubricated and build up on that surface to form multimolecular layers. The carrier may be a liquid such as an oil or grease or may even be aqueous. Solid carriers are also feasible such as polyamide plastics such as those used to build up worn machinery parts such as drive shafts and the like. Incorporation of a heteropolar compound in the plastic material enables a multimolecular layer of heteropolar molecules to form not only on the surface of the plastic by migration through the plastic material but also by transfer from the surface of the plastic to another surface which rubs against the surface of the plastic.

It has also been found that the heteropolar molecules migrate laterally over the surface on which they are adsorbed beyond the boundaries of contact of that surface with the carrier material. Contact of the carrier with the whole of the surface to be protected is not therefore necessary in order to form a lubricating layer of heteropolar molecules over all the surface to be protected. Nor is it necessary to have continuous contact between carrier and surface to be treated, but intermittent contact is also effective. The multimolecular layer is not of course formed instantaneously but builds up over a period of time. Relative movement of carrier and surface to be protected accelerate the formation and maintainance of the multimolecular layer of heteropolar molecules on the surface to be protected.

The heteropolar molecules migrate through the carrier to the interfaces of the carrier with the surrounding environment. Unsubstituted heteropolar heterocyclic unsaturated single or condensed ring systems having the aforementioned hydrogen donor and acceptor moieties have this property of migration. Any substituents in such heteropolar molecules should not exert such a solubilizing effect on the heteropolar molecules that they lose their ability to migrate through the carrier to the interfaces of the carrier's environment. Since a major application of the compounds of the invention is in oils and greases it is essential that the molecules should not exert such a solubilizing effect that they fail to migrate. Consequently, where they are to be added to oils and greases any substituted groupings should not "over solubilize" the molecule. Therefore hydrocarbon substituents should preferably not contain more than 4 carbon atoms, preferably not more than 2 carbon atoms.

The carrier may be a liquid such as a lubricating oil or hydrocarbon fuel for an internal combustion engine or aqueous system, or the carrier may be a grease or semi-solid material (non-Newtonian fluid) such as a lubricating grease or grease-like lubricant. The carrier may also be a solid such as a plastics composite, e.g. a polyamide used in repairing or rebuilding beading surfaces. In the case of liquid the content of heteropolar compound may be from 0.5% to 4% by weight based on the total weight of carrier and additive and in the case of greases or non-Newtonian fluids may be from 3% to 10% by weight based on the total weight of carrier plus additive. Preferably, in the case of a liquid the content of heteropolar compound is greater than 1%, e.g. from 1.1% to 4% by weight based on the total weight of carrier and additive. The concentration necessary in a solid carrier will depend on the type of solid carrier involved. In the case of polyamides somewhat more additive is in general necessary than that required in a semi-solid for equivalent results. This is the case of a 'Polyamid' bearing 10% by weight based on the total weight of 'Polyamid" and additive was found satisfactory. However amounts of greater than 10% e.g. 10.1% to 20% are preferred.

The preferred hydrogen acceptor moiety is one involving nitrogen as the heteroatom in the form of an -N = moiety. The preferred hydrogen donor moiety is a hydroxyl group. Both such moieties occur in the preferred heteropolar compound of the invention which is 8-hydroxyquinoline:- The condensed ring system in the heteropolar compounds useful in the invention may contain up to four -N = moieties, with preferably up to two such moieties being incorporated as ring forming atoms in any one ring. Other unsubstituted heteropolar compounds useful in the method and compositions of the present invention include:

As previously indicated the preferred heteropolar compounds are unsubstitued materials. Substituents should not create steric hindrance which prevents interaction of the hydrogen donor and acceptor moieties. Thus the provision of a methyl group ortho to the -N = hydrogen acceptor moiety of 8-hydroxyquinoline to form the compound:- does not materially affect the activity of this heteropolar molecule in forming adsorption film on metal surfaces. The number and size of the substituents which can be tolerated in the heteropolar molecule depends on the number and position of the hydrogen donor and acceptor moieties in the molecule. In general the substituents groups should not exceed four atoms in number (e.g. in the case of hydrocarbyl the butyl group), preferably no more than two atoms and more preferably still only one carbon atom.

A good indication of whether steric hindrance is likely to cause problems is given by measuring the adsorption-free energy of the compound in question. If the adsorption-free energy as measured on a copper surface is substantially in the range of 3 to 6 Kcal/mol then steric hindrance is unlikely to be a problem.

The invention will be further illustrated by reference to the following Examples which are purely illustrative. In each of the examples the heteropolar compound was 8-hydroxyquinoline.

### EXAMPLE 1

0.5% by weight of heteropolar compound was incorporated in SAE 30 engine oil which was then used in a test-bed fully instrumented Whirlepeel system. The following results were obtained as shown in Tables 1 to 5.

The following Examples show the EP effect of adding the heteropolar compound to different lubricants.

### EXAMPLE 2

### EXTREME PRESSURE (EP) EFFECT

Shell Four Ball Machine Lubricating Medium: Lithium grease, with 3% by weight of heteropolar compound. WITHOUT HETEROPOLAR welding at 2^{7 -} 2.27 N WITH HETEROPOLAR no welding at 3⁷N

### EXAMPLE 3

### FALEX LUBRICANTS TESTER

To. L.P. Test 241/69 with 0.5% by weight of heteropolar compound.

### EXAMPLE 4

### COMPOSITE MATERIALS

'Polyamid' Bearing with 10% of MₒS₂ composite additive, compared with a similar bearing containing 10% of heteropolar compound. The bearing having the heteropolar compound in the 'Polyamid' lowered the friction by 30% as compound to the bearing containing the MₒS₂ additive.

### EXAMPLE 5

### NOISE REDUCTION

When the heteropolar compound was incorporated in the lubricant in a back axle differential gearing the noise reduced by 2dB. When the heteropolar compound was incorporated in the lubricant in a Vauxhall Astra engine the noise decreased by 86dB to 80dB.

## Claims

1. A method of reducing wear on a surface which is subject to frictional forces which comprises forming and maintaining on said surface a protective layer characterised in that said protective layer is a multi- molecular layer of a heteropolar compound comprising at least one wholly unsaturated heterocyclic six-membered ring in which at least one unsubstituted heteroatom moiety acts as a hydrogen acceptor and in which said compound also comprises at least one hydrogen donor moiety, and in which said heteropolar compound has no substituent which by itself or together with another substituent or substituents creates such steric hindrance and/or renders the molecule so basic or acidic or so alters the steric geometry of the molecule as to prevent interaction of the hydrogen donor and acceptor moieties of one molecule of the heteropolar compound with the hydrogen donor and acceptor moieties of another molecule of said heteropolar compound nor any substituent which by itself or together with another substituent or substituents has the effect of solubilizing said heteropolar compound in a selected carrier to the extent that migration of the heteropolar compound to the interfaces of the carrier with the carrier environment is prevented and in which the protective layer is formed on the surface to be protected by contacting at least a portion of the said surface with a composition comprising a carrier and dissolved and/or dispersed therein an effective amount of said heteropolar compound.

2. A method as claimed in claim 1, in which at least a portion of the surface to be protected is continuously contacted with said composition.

3. A method as claimed in claim 1, in which at least a portion of the surface to be protected in intermittently contacted with said composition.

4. A method as claimed in any of claims 1 to 3, characterised in that the heteropolar compound comprises up to three condensed unsaturated rings, one of which rings is said wholly unsaturated heterocyclic six-membered ring.

5. A method as claimed in claim 4, characterised in that one of said condensed rings is a five-membered unsaturated heterocyclic ring.

6. A method as claimed in claim 4, characterised in that all the condensed rings are six-membered unsaturated rings.

7. A method as claimed in any of claims 1 to 6, in which the carrier is a liquid.

8. A method as claimed in claim 7, characterised in that the liquid is a lubricating oil.

9. A method as claimed in claim 8, characterised in that the lubricating oil comprises at least one unsaturated hydrocarbon.

10. A method as claimed in claim 9, characterised in that the heteropolar compound is present in the range 1.1 % to 4% by weight based on the total weight of carrier and additive.

11. A method as claimed in claim 7, characterised in that the carrier is an aqueous liquid.

12. A method as claimed in claim 7, characterised in that the carrier is a liquid hydrocarbon fuel for an internal combustion engine.

13. A method as claimed in any of claims 1 to 6, characterised in that the carrier is a lubricating grease or grease-like material.

14. A method as claimed in claim 13, characterised in that the heteropolar compound is present in the range 3% to 10% by weight based on the total weight of carrier and additive.

15. A method as claimed in any of claims 1 to 6, characterised in that the carrier is a solid plastics material.

16. A method as claimed in claim 15, characterised in that the solid plastics material is a polyamide.

17. A method as claimed in claim 16, characterised in that the heteropolar compound is present in the range 10.1 % to 20% based on the total weight of carrier and additive.

18. A method as claimed in any of the preceding claims, characterised in that the heterocyclic moiety which acts as a hydrogen acceptor is an -N = moiety.

19. A method as claimed in claim 18, characterised in that the heteropolar compound contains up to four -N = moieties.

18. A method as claimed in any of the preceding claims, characterised in that the hydrogen donor moiety is an -OH group.

21. A method as claimed in any of the preceding claims, characterised in that the heteropolar compound is 8-hydroxyquinoline.

22. A method as claimed in any of claims 1 to 20, characterised in that the heteropolar compound is selected from 2,3-dihydroxypyridine, 4,6-dihydroxypyrinidine, 2-pteridinol, 2-methyl 8-quinolinol, 2,4-quinolindiol, 2,3-dihydroxyquinoxalin, 2,4-pteridinediol, 6-purinol, 3-phenanthridinol, 2-phenanthrolinol and 2-phenazinol.

## Patentansprüche

1. Verfahren zur Verminderung des Verschleißes auf einer Oberfläche, die Reibungskräften ausgesetzt ist, das die Bildung einer Schutzschicht und deren Aufrechterhaltung auf der Oberfläche umfaßt, dadurch gekennzeichnet, daß die Schutzschicht eine Multimolekularschicht aus einer heteropolaren Verbindung ist, die wenigstens einen vollständig ungesättigten heterocyclischen sechsgliedrigen Ring umfaßt, bei dem wenigstens ein unsubstituiertes Heteroatomfragment als Wasserstoffakzeptor fungiert, die Verbindung auch noch zumindest ein Wasserstoffdonatorfragment umfaßt, und die heteropolare Verbindung keinen Substituenten aufweist, der als solcher oder zusammen mit einem anderen Substituenten oder anderen Substituenten eine solche sterische Behinderung bewirkt und/oder das Molekül so basisch oder sauer macht oder die sterische Geometrie des Moleküls so verändert, daß eine Wechselwirkung zwischen dem Wasserstoffdonator- und -akzeptorfragment eines Moleküls der heteropolaren Verbindung mit dem Wasserstoffdonator- und -akzeptorfragment eines anderen Moleküls der heteropolaren Verbindung verhindert wird, und auch keinen Substituenten, der als solcher oder zusammen mit einem anderen Substituenten oder anderen Substitutenten die heteropolare Verbindung in einem ausgewählten Träger soweit solubilisiert, daß die Wanderung der heteropolaren Verbindung zu den Grenzflächen zwischen dem Träger und seiner Umgebung verhindert wird und bei dem die Schutzschicht auf der zu schützenden Oberfläche durch Kontaktierung wenigstens eines Teils der Oberfläche mit einem Gemisch gebildet wird, das einen Träger und eine darin gelöste und/oder dispergierte wirksame Menge der heteropolaren Verbindung enthält.

2. Verfahren nach Anspruch 1, wobei wenigstens ein Teil der zu schützenden Oberfläche ständig mit dem Gemisch in Berührung gebracht wird.

3. Verfahren nach Anspruch 1, wobei wenigstens ein Teil der zu schützenden Oberfläche periodisch mit dem Gemisch in Berührung gebracht wird.

4. Verfahren nach einem der Ansprüche 1 bis 3, dadurch gekennzeichnet, daß die heteropolare Verbindung bis zu drei kondensierte ungesättigte Ringe umfaßt, von denen einer der vollständig ungesättigte heterocyclische sechsgliedrige Ring ist.

5. Verfahren nach Anspruch 4, dadurch gekennzeichnet, daß einer der kondensierten Ringe ein fünfgliedriger ungesättiger heterocyclischer Ring ist.

6. Verfahren nach Anspruch 4, dadurch gekennzeichnet, daß alle kondensierten Ringe sechsgliedrige ungesättigte Ringe sind.

7. Verfahren nach einem der Ansprüche 1 bis 6, wobei der Träger eine Flüssigkeit ist.

8. Verfahren nach Anspruch 7, dadurch gekennzeichnet, daß die Flüssigkeit ein Schmieröl ist.

9. Verfahren nach Anspruch 8, dadurch gekennzeichnet, daß das Schmieröl wenigstens einen ungesättigten Kohlenwasserstoff umfaßt.

10. Verfahren nach Anspruch 9, dadurch gekennzeichnet, daß die heteropolare Verbindung in einer Menge von 1,1 bis 4 Gew.-%, bezogen auf das Gesamtgewicht von Träger und Zusatz, vorliegt.

11. Verfahren nach Anspruch 7, dadurch gekennzeichnet, daß der Träger eine wässerige Flüssigkeit ist.

12. Verfahren nach Anspruch 7, dadurch gekennzeichnet, daß der Träger ein flüssiger Kohlenwasserstoff-Kraftstoff für einen Verbrennungsmotor ist.

13. Verfahren nach einem der Ansprüche 1 bis 6, dadurch gekennzeichnet, daß der Träger ein Schmierfett oder ein fettähnlicher Stoff ist.

14. Verfahren nach Anspruch 13, dadurch gekennzeichnet, daß die heteropolare Verbindung in einer Menge von 3 bis 10 Gew.-%, bezogen auf das Gesamtgewicht von Träger und Zusatz, vorliegt.

15. Verfahren nach einem der Ansprüche 1 bis 6, dadurch gekennzeichnet, daß der Träger ein fester Kunststoff ist.

16. Verfahren nach Anspruch 15, dadurch gekennzeichnet, daß der feste Kunststoff ein Polyamid ist.

17. Verfahren nach Anspruch 16, dadurch gekennzeichnet, daß die heteropolare Verbindung in einer Menge von 10,1 bis 20 Gew.-%, bezogen auf das Gesamtgewicht von Träger und Zusatz, vorliegt.

18. Verfahren nach einem der vorangegangenen Ansprüche, dadurch gekennzeichnet, daß der als Wasserstoffakzeptor fungierende heterocyclische Anteil ein -N =-Fragment ist.

19. Verfahren nach Anspruch 18, dadurch gekennzeichnet, daß die heteropolare Verbindung bis zu vier -N =-Fragmente enthält.

20. Verfahren nach einem der vorangegangenen Ansprüche, dadurch gekennzeichnet, daß der Wasserstoffdonatoranteil eine -OH-Gruppe ist.

21. Verfahren nach einem der vorangegangenen Ansprüche, dadurch gekennzeichnet, daß die heteropolare Verbindung 8-Hydroxychinolin ist.

22. Verfahren nach einem der Ansprüche 1 bis 20, dadurch gekennzeichnet, daß die heteropolare Verbindung ausgewählt wird unter 2,3-Dihydroxypyridin, 4,6-Dihydroxypyrinidin, 2-Pteridinol, 2-Methyl-8-chinolinol, 2,4-Chinolindiol, 2,3-Dihydroxychinoxalin, 2,4-Pteridindiol, 6-Purinol, 3-Phenanthridinol, 2-Phenanthrolinol und 2-Phenazinol.

## Revendications

1. Procédé pour réduire l'usure sur une surface qui est soumise à des forces de frottement, qui consiste à former et maintenir une couche protectrice sur ladite surface, caractérisé en ce que ladite couche protectrice est une couche polymoléculaire d'un composé hétéropolaire comprenant au moins un hétérocycle hexagonal insaturé dans lequel au moins un fragment hétéroatomique entièrement non substitué agit comme accepteur d'hydrogène et dans lequel ledit composé comprend également au moins un fragment donneur d'hydrogène, et dans lequel ledit composé hétéropolaire ne porte aucun substituant qui, par lui-même ou conjointement à un ou plusieurs autres substituants, crée un empêchement stérique et/ou rend la molécule basique ou acide ou altère la géométrie stérique de la molécule à tel point que cela empêche une interaction des fragments donneur et accepteur d'hydrogène d'une molécule du composé hétéropolaire avec les fragments donneur et accepteur d'hydrogène d'une autre molécule dudit composé hétéropolaire, ni aucun substituant qui, par lui-même ou conjointement à un ou plusieurs autres substituants, a pour effet de solubiliser ledit composé hétéropolaire dans un support choisi à tel point que soit empêchée la migration du composé hétéropolaire vers les interfaces entre le support et l'environnement du support, et dans lequel la couche protectrice est formée sur la surface à protéger par la mise en contact d'au moins une partie de ladite surface avec une composition comprenant un support et une quantité efficace dudit composé hétéropolaire dissous et/ou dispersé dans celui-ci.

2. Procédé tel que revendiqué dans la revendication 1, dans lequel au moins une partie de la surface à protéger est mise en contact de façon continue avec ladite composition.

3. Procédé tel que revendiqué dans la revendication 1, dans lequel au moins une partie de la surface à protéger est mise en contact de façon intermittente avec ladite composition.

4. Procédé tel que revendiqué dans l'une quelconque des revendications 1 à 3, caractérisé par le fait que le composé hétéropolaire comprend jusqu'à trois cycles insaturés condensés, dont l'un est l'hétérocycle hexagonal entièrement insaturé.

5. Procédé tel que revendiqué dans la revendication 4, caractérisé par le fait que l'un desdits cycles condensés est un hétérocycle insaturé pentagonal.

6. Procédé tel que revendiqué dans la revendication 4, caractérisé par le fait que tous les cycles condensés sont des cycles insaturés hexagonaux.

7. Procédé tel que revendiqué dans l'une quelconque des revendications 1 à 6, dans lequel le support est un liquide.

8. Procédé tel que revendiqué dans la revendication 7, caractérisé par le fait que le liquide est une huile lubrifiante.

9. Procédé tel que revendiqué dans la revendication 8, caractérisé par le fait que l'huile lubrifiante comprend au moins un hydrocarbure insaturé.

10. Procédé tel que revendiqué dans la revendication 9, caractérisé par le fait que le composé hétéropolaire est présent dans l'intervalle de 1,1 % à 4 % en poids par rapport au poids total de support et d'additif.

11. Procédé tel que revendiqué dans la revendication 7, caractérisé par le fait que le support est un liquide aqueux.

12. Procédé tel que revendiqué dans la revendication 7, caractérisé par le fait que le support est un combustible hydrocarboné liquide pour moteur à combustion interne.

13. Procédé tel que revendiqué dans l'une quelconque des revendications 1 à 6, caractérisé par le fait que le support est une graisse lubrifiante ou une matière lubrifiante semblable à une graisse.

14. Procédé tel que revendiqué dans la revendication 13, caractérisé par le fait que le composé hétéropolaire est présent dans l'intervalle de 3 % à 10 % en poids par rapport au poids total de support et d'additif.

15. Procédé tel que revendiqué dans l'une quelconque des revendications 1 à 6, caractérisé par le fait que le support est une matière plastique solide.

16. Procédé tel que revendiqué dans la revendication 15, caractérisé par le fait que la matière plastique solide est un polyamide.

17. Procédé tel que revendiqué dans la revendication 16, caractérisé par le fait que le composé hétéropolaire est présent dans l'intervalle de 10,1 % à 20 % par rapport au poids total de support et d'additif.

18. Procédé tel que revendiqué dans l'une quelconque des revendications précédentes, caractérisé par le fait que le fragment hétérocyclique qui agit comme accepteur d'hydrogène est un chaînon -N = .

19. Procédé tel que revendiqué dans la revendication 18, caractérisé par le fait que le composé hétéropolaire contient jusqu'à quatre chaînons -N = .

20. Procédé tel que revendiqué dans l'une quelconque des revendications précédentes, caractérisé par le fait que le fragment donneur d'hydrogène est un groupe -OH.

21. Procédé tel que revendiqué dans l'une quelconque des revendications précédentes, caractérisé par le fait que le composé hétéropolaire est la 8-hydroxyquinoléine.

22. Procédé tel que revendiqué dans l'une quelconque des revendications 1 à 20, caractérisé par le fait que le composé hétéropolaire est choisi parmi la 2,3-dihydroxypyridine, la 4,6-dihydroxypyrimidine, le 2-ptéridinol, le 2-méthyl-8-quinolinol, le 2,4-quinolinediol, la 2,3-dihydroxyquinoxaline, le 2,4-ptéridine- diol, le 6-purinol, le 3-phénanthridinol, le 2-phénanthrolinol et le 2-phénazinol.
